

## UNITED STATES PATENT OFFICE

1,953,997

## ANODIC COATING OF ZINC BASE METALS

Edward Cushman Truesdale and Ernest John  
Wilhelm, Palmerton, Pa., assignors to The New  
Jersey Zinc Company, New York, N. Y., a cor-  
poration of New Jersey

No Drawing. Application November 14, 1932,  
Serial No. 642,608

14 Claims. (Cl. 204—1)

This invention relates to the coating of zinc base metals by anodic action, and has for its object the provision of an improved method of producing useful anodic coatings on such metals, as well as the provision, as new articles of commerce, of zinc base metals so coated. By "zinc base metal" we mean metals and alloys composed principally of zinc.

The invention is particularly concerned with the production of anodic coatings on zinc and zinc base alloys for the purpose of protection, ornamentation, or of serving as a base for the application of paints, lacquers and the like so as to secure good adhesion of the latter. Ordinary commercial zinc (in particular, rolled or strip zinc), zinc base alloys such as die-casting alloys containing over 90% zinc (for example, the alloys of United States Patents Nos. 1,596,761, 1,663,215, 1,779,525, 1,852,434, 1,852,441 and 1,852,442), and wrought zinc base alloys (for example, the alloys of United States Patents Nos. 1,716,599, 1,832,653, 1,832,733 and 1,835,450) may be advantageously coated by the method of the invention. Numerous other zinc base alloys, particularly those containing small amounts of copper and/or aluminum, are likewise amenable to treatment in accordance with the invention.

Anodic coatings have heretofore been produced on metals by subjecting the metal as anode to electrolytic treatment. So far as we are aware, however, no practical and commercially satisfactory method has heretofore been available for the production of useful anodic coatings on zinc base metals. As the result of an exhaustive investigation of the subject we have discovered that dense and firmly adherent anodic coatings can be produced on zinc base metals from strongly basic electrolytes. Thus, we have found that with a strongly alkaline electrolyte, having a hydroxyl ion concentration corresponding to a pH value of about 13.3 or greater, highly useful coatings can be produced on zinc anodes under appropriate conditions of voltage, current density and temperature. Based on these discoveries, our present invention involves, in its broad aspect, producing an anodic coating on a zinc base metal by subjecting the metal as anode to electrolytic treatment in an alkaline electrolyte of high hydroxyl ion concentration. The hydroxyl ion concentration should not be so high as to dissolve as zincate all of the zinc compounds formed anodically, and preferably the electrolyte should not contain anions that form water-soluble compounds with zinc (such as anions of acetic acid, or of strong acids like sulphuric acid and hydrochloric acid).

A satisfactory electrolyte for the practice of the invention is an aqueous solution of a hydroxide of an alkali metal or alkaline earth metal, for example, caustic soda, caustic potash and barium hydroxide, having a pH value of about 13.3. 60

In carrying out the invention, the articles of zinc or zinc base alloys to be coated are subjected to an electrolytic treatment as anode while immersed in an electrolyte of high hydroxyl ion concentration. When so treated at appropriate voltages, current densities and temperatures, the zinc articles become coated with a firm adherent layer of zinc oxide and/or hydrated zinc oxide formed by reaction of zinc and hydroxyl ions. The coatings are dark in color, commonly blue-black, and possess a pleasing lustre and iridescence. 65

The coatings ordinarily produced on zinc by corrosion in solution (e. g. alkaline solutions) are in general relatively loose and poorly adherent. In contrast with this, the anodic coatings produced in accordance with the present invention are thin, dense and firmly adherent. These anodic coatings usually reproduce in minute detail the surface markings originally present on the treated metal objects. This is probably due 70 to the fact that the coating is formed primarily by reaction of the hydroxyl ions discharged at the anode with zinc atoms in situ in the crystallites of the zinc metal. On the other hand, it is possible that the coating is formed in whole or in 75 part by reaction of hydroxyl ions with zinc ions in solution in the electrolyte at the surface of the anode, followed by precipitation upon the anode of the insoluble zinc compound thus formed. The X-ray patterns of the coatings indicate that they 80 consist essentially of zinc oxide. 90

Since the anodic coating of the invention usually reproduces, in minute detail, the surface markings originally present on the zinc article, the appearance of the coating may be improved 95 by buffing the zinc article before anodic treatment. This buffing procedure may advantageously be of the same character as used on zinc prior to electro-plating. Other preliminary treatment, such as sand-blasting or etching 100 which, like buffing, removes a surface film especially likely to be present on cast zinc surfaces, may be employed to facilitate the subsequent anodic treatment. Such preliminary surface treatment of the zinc article may, of course, be 105 dispensed with if desired.

The zinc article should be appropriately cleaned prior to anodic treatment. This cleaning may be advantageously accomplished in a trisodium phosphate solution containing about six ounces 110

per gallon of water (45 grams per liter of water). This solution is used hot as an electro-cleaner, with the zinc article to be cleaned as the cathode, and with sufficient current to produce copious 5 gassing. When used in this manner, grease (e. g. acquired during rolling or buffing) and loose dirt are completely removed after one-half to three minutes of cleaning. After cleaning, the zinc article is rinsed in hot and then in cold water 10 to remove the residual cleaning solution, following which the zinc article is ready for anodic treatment.

A very satisfactory electrolyte for the practice of the invention is an 0.5N aqueous solution of 15 sodium hydroxide. The electrolytic treatment is conducted at room temperature with a current density at the anode of from 10 to 60 amperes per square foot, and with a duration of treatment of from 1 to 15 minutes. Under these operating 20 conditions, dark, usually blue-black, coatings are obtained on anodes of zinc and of zinc base alloys of the types hereinbefore mentioned. The coatings are firmly adherent, uniform in color and duplicate the minute markings on the original surface in every detail. The coatings may 25 be given a high lustre by buffing. If entirely black coatings are desired, the films may be dyed with nigrosine or the like.

The specified operating conditions may be 30 varied without departing from the spirit and scope of the invention. Thus, the concentration of the sodium hydroxide solution may be varied from 0.2N to 1.0N without changing the essential properties of the anodic deposit. The current 35 density may likewise be varied, but the use of current densities less than 10 amperes per square foot requires an unnecessarily long time of treatment while the use of current densities above 60 amperes per square foot results in the use of an 40 unnecessarily high current. A 6 to 12 volt source of electric energy is sufficient. Technical flake sodium hydroxide is sufficiently pure for the purpose. The cathode used in the electrolytic treatment may be of nickel, iron or other metal in- 45 soluble in sodium hydroxide solution.

A saturated solution of barium hydroxide is also a satisfactory electrolyte for the practice of the invention. Under the same operating conditions as hereinbefore described, and with a barium hydroxide electrolyte saturated at room 50 temperature (the operating temperature), anodic films are produced of the same character as obtained with the 0.5N sodium hydroxide solution. Barium hydroxide can be added to sodium hydroxide electrolytes without altering the nature 55 of the anodic coatings obtained therefrom. Thus, if it is desired to keep a sodium hydroxide electrolyte free from sodium carbonate formed by absorption of carbon dioxide from the air, barium 60 hydroxide may be added to precipitate any soluble carbonate as barium carbonate.

During the anodic treatment, some zinc goes into solution in the strongly alkaline electrolyte. Loss in weight of the zinc anode has been determined as a function of the current density and time of treatment, and while such losses are not more than 1 or 2 grams per square foot, on the average, they are found to decrease as the current density is increased, for a given quantity 70 of current flowing. This small amount of zinc enters solution as zincate ions, with which a low concentration of zinc ions are in equilibrium, as is shown by the fact that a small amount of zinc is deposited electrolytically at the cathode. The 75 electrolyte actually present during the operation

thus contains a small amount of zinc (e. g. sodium zincate) as well as sodium hydroxide. The presence of this zinc in solution in the electrolyte exercises no deleterious influence on the anodic treatment so long as the hydroxyl ion concentration of the electrolyte corresponds to a pH value of about 13.3 or higher. Similarly, with this high hydroxyl ion concentration (pH of 13.3 or greater), the electrolyte may contain, by contamination or otherwise, small amounts 80 of other dissolved substances. 85

The anodic coatings of the invention not only protect the zinc or zinc alloy from corrosion, but are also useful for decoration. These coatings 90 may also be used as a base to increase the adherence of paint, enamel, lacquer, etc. Anodic coatings produced in accordance with the invention, although composed for the most part, if not entirely, of zinc oxide, are dark, commonly blue-black in color. The coating may be dyed jet black by nigrosine, or similar dye. The dyeing may take place during the electrolytic treatment by solution of the dye in the electrolyte, or dyeing may be carried out by immersion 95 of the coated article in a solution of the dye. 100

We claim:

1. As a new article of commerce, a zinc base metal having a dark-colored, thin, dense and firmly adherent anodic coating composed essentially of zinc oxide. 105

2. As a new article of commerce a zinc base metal having a blue-black, thin, dense and firmly adherent anodic coating composed essentially of zinc oxide.

3. The method of producing a coating on a zinc base metal which comprises subjecting the metal as anode to electrolytic treatment in an alkaline electrolyte having a pH of about 13.3 or greater.

4. The method of producing a coating on a zinc base metal which comprises subjecting the metal as anode to electrolytic treatment in an alkaline electrolyte having a hydroxyl ion concentration greater than the equivalent of a 0.2N sodium hydroxide solution. 115

5. The method of producing a coating on a zinc base metal which comprises subjecting the metal as anode to electrolytic treatment in an alkaline electrolyte having a concentration of free alkali not less than the equivalent of a 0.2N sodium hydroxide solution. 120

6. The method of producing a coating on a zinc base metal which comprises subjecting the metal as anode to electrolytic treatment in an alkaline electrolyte with a high hydroxyl ion concentration that is adapted to produce an anodic coating on the zinc metal that is dark in color, firmly adherent and composed for the most part of zinc oxide. 130

7. The method of producing a coating on a zinc base metal which comprises subjecting the metal as anode to electrolytic treatment in an alkaline electrolyte with a high hydroxyl ion concentration that is adapted to produce an anodic coating on the zinc metal that is blue-black in color, firmly adherent and composed for the most part of zinc oxide. 135

8. The method of producing a coating on a zinc base metal which comprises subjecting the metal as anode to electrolytic treatment at a current density of from 10 to 60 amperes per square foot of anode surface in an alkaline electrolyte having a pH of about 13.3 or greater. 145

9. The method of producing a coating on a zinc base metal which comprises subjecting the metal 150

as anode to electrolytic treatment for from 1 to 15 minutes at a current density of from 10 to 60 amperes per square foot in an alkaline electrolyte having a pH of about 13.3 or greater.

5 10. The method of producing a coating on a zinc base metal which comprises subjecting the metal as anode to electrolytic treatment in a 0.2N to 1.0N solution of sodium hydroxide.

10 11. The method of producing a coating on a zinc base metal which comprises subjecting the metal as anode to electrolytic treatment in a solution of sodium hydroxide having a concentration of about 0.5N NaOH.

12. The method of producing a coating on a zinc base metal which comprises subjecting the metal as anode to electrolytic treatment at a

current density of from 10 to 60 amperes per square foot of anode surface in a 0.2N to 1.0N solution of sodium hydroxide.

13. The method of producing a coating on a zinc base metal which comprises subjecting the metal as anode to electrolytic treatment in a substantially saturated solution of barium hydroxide.

14. The method of producing a coating on a zinc base metal which comprises subjecting the metal as anode to electrolytic treatment in an alkaline electrolyte containing sodium hydroxide and barium hydroxide and having a pH of about 13.3 or greater.

EDWARD CUSHMAN TRUESDALE. 90  
ERNEST JOHN WILHELM. 90

20 95

25 100

30 105

35 110

40 115

45 120

50 125

55 130

60 135

65 140

70 145

75 150